

F. J. TONE.  
REDUCTION OF REFRACTORY ORES.  
APPLICATION FILED APR. 8, 1907.

1,028,151.

Patented June 4, 1912.



WITNESSES

R. A. Balderson  
G. B. Fleming

INVENTOR

Frank J. Tone  
by Lawrence Bynes  
his attorney

# UNITED STATES PATENT OFFICE.

FRANK J. TONE, OF NIAGARA FALLS, NEW YORK.

## REDUCTION OF REFRactory ORES.

1,028,151.

Specification of Letters Patent.

Patented June 4, 1912.

Application filed April 8, 1907. Serial No. 366,915.

To all whom it may concern:

Be it known that I, FRANK J. TONE, of Niagara Falls, Niagara county, New York, have invented a new and useful Improvement in the Reduction of Refractory Ores, of which the following is a full, clear, and exact description, reference being had to the accompanying drawing, forming part of this specification, in which the figure is a 10 sectional side elevation showing one form of electric furnace for carrying out my invention.

The invention relates to reducing of refractory compounds in the electric furnace, and particularly those compounds which are more or less volatile at the temperature of reduction.

The object of the invention is to reduce the loss and thereby increase the efficiency 20 in the electric furnace reduction.

While the process is generally applicable to refractory ores or compounds, particularly those which are volatile at their reduction temperatures; I will describe my invention particularly with reference to the reduction of silica compounds for the manufacture of silicon, silicon alloys and sili- 25 cides.

Heretofore in the production of silicon, 30 it has been customary to employ a mixture of carbon and silica in the proper proportions, the product of the reaction in the electric furnace being silicon and carbon monoxid gas. During this process the evolution 35 of the carbon and monoxid gas is rapid, and tends to carry out of the furnace a certain proportion of vapor of silicon and silicon compounds, thus reducing the output and lowering the efficiency. This loss by volatilization is the 40 most serious of all losses taking place during the process. I have discovered that these losses by volatilization can be greatly reduced by confining the gases in the furnace and releasing them only at or above a certain normal pressure. The furnace may be constructed in many different ways for accomplishing this desired result. I prefer, however, to inclose the furnace by suitable 45 means to make it impervious and to provide outlets having means for releasing the gases when the pressure reaches or exceeds a certain predetermined amount.

In the drawing, I show an ordinary type 50 of arc furnace, having a crucible 1 making

up the side walls and bottom, and provided with a tight cover 2. This cover fits closely around the electrode 3 and upon the side walls. 4 represents the other electrode, which is preferably mounted upon a carbon 60 base block 5, constituting the other terminal of the furnace.

6 is a charging hopper, having a raising and lowering bell, or other suitable means for feeding the charge into the furnace, and 65 7 is a weighted valve normally closing a gas exit through the top or cover. One or more of these controlled gas outlets may be provided, by which the exit of the gases and volatile products may be controlled and 70 their pressure thus regulated. The charge of the furnace is shown at 8, 9 being the usual tap hole at the bottom.

In the operation of the furnace, the zone of reaction formed by the arc, or otherwise, 75 may be surrounded by a considerable body of charged material in a finely ground non-porous state, or of such character that the exit of the gases is impeded; and in this way it is possible to raise the pressure of 80 the gases in the reaction zone to a considerable amount above their normal pressure. Silica has an appreciable vapor tension, even below the point at which it fuses and 85 below the point of reduction; and by increasing the pressure in the reduction zone, the vaporizing point of the silica and reduced silicon is raised, resulting in preventing to a large extent the volatilizing of the 90 products. The condensation of the volatile products is also assisted.

The process may be applied to reducing other elements, subject to volatilization losses, such as aluminum, manganese boron, &c.

Many changes may be made in the form 95 and arrangement of the furnace, &c., without departing from my invention.

I claim:

1. The method of reducing metallic compounds subject to volatilization losses, consisting in electrically heating a mixture of the compound and a reducing agent within the reduction zone of an electric arc furnace to a temperature sufficient to cause volatilization of the compound and its reduction by the reducing agent, and maintaining the gases in the reduction zone under a raised pressure sufficient to reduce volatilization losses and to promote condensation of the reduced product but insufficient to wholly 105 110 115

prevent volatilization of the compounds of the charge.

2. The process of reducing silicon compounds subject to volatilization losses, consisting in electrically heating a mixture of the compound and a reducing agent within the reduction zone of an electric arc furnace to a temperature sufficient to cause volatilization of the compound and its reduction by 10 the reducing agent, and maintaining the gases in the reduction zone under a raised

pressure sufficient to reduce volatilization losses and to promote condensation of the reduced product but insufficient to wholly prevent volatilization of the compounds of 15 the charge.

In testimony whereof, I have hereunto set my hand.

FRANK J. TONE.

Witnesses:

F. I. PIERCE,  
CHARLES CHORMANN.